# EUROPEAN PATENT SPECIFICATION

(11) **EP 0 158 387 B1**
(45) Date of publication and mention of the grant of the patent: **27.12.1989**
(21) Application number: 85200407.6
(22) Date of filing: 18.03.1985
(51) Int. Cl.: C10L 9/08

(54) **A process for calcining green coke**
Verfahren zur Kalzinierung von grünem Koks
Procédé pour la calcination de coke vert

(30) Priority: 11.04.1984 GB 8409402
(43) Date of publication of application: 16.10.1985
(73) Proprietor: SHELL INTERNATIONALE RESEARCH MAATSCHAPPIJ B.V., 2596 HR Den Haag (NL)
(72) Inventor: Lindhout, Izaak, NL-2596 HR The Hague (NL); Geiger, Ferdinand Johan Adriaan, NL-2596 HR The Hague (NL); Alberts, Barend, NL-2596 HR The Hague (NL); Downing, Roger Stewart, NL-1031 CM The Hague (NL)
(74) Representative: Aalbers, Onno

(56) References cited:
- FR-A- 1 555 005
- FR-A- 2 396 062
- GB-A- 2 043 676
- US-A- 3 677 533
- US-A- 4 160 814

## Description

The invention relates to a process for calcining green coke containing combustible volatile matter in at least two stages, whereby in a first stage the green coke is heated in a furnace to a temperature of between 750°C and 1000°C and in a second stage in a second furnace to a temperature of between 1200°C and 1600°C.

It is generally known that green coke made from a suitable hydrocarbon feedstock may be converted to high quality needle coke for use in high performance graphite electrodes which are applied in electric ore furnaces, or other purposes, like in baked carbon anodes in aluminium cells. For this purpose the green coke, after the water being removed at relatively low temperatures, is heated (precalcinated) in a furnace to a temperature which necessary to release at least a part of the combustible volatile matter, generally around 800°C. In a further stage the coke is calcined in a second furnace to a temperature in the range between 1200°C and 1600°C. In principle in each of the stages either a shaft kiln, a rotary kiln or a rotary hearth furnace may be used, depending on the specific circumstances. After the precalcination cooling of the product may optionally take place, before the second stage calcination is carried out. The patent literature describes a number of processes for calcining coke, for example UK Patent Specification 1,603,924, UK Patent Applications 2,093,061 and 2,016,512, German Patent Specification 2,931,475 and US Patent Specification 4,291,008.

In UK Patent Specification 1,603,924 is disclosed a process for calcining green coke in three stages of heating furnaces which are connected in series and in which process in a first step the water is evaporated from the green coke, in a second step the volatile matter is distilled off and burnt from the dried coke and in a third step the coke is calcined. In the precalcination stage preheated air is introduced into the burning kiln in order to burn the released volatile matter. Disadvantages are the degradation in particle size distribution upon calcination, the high friability of the product obtained by such a process and the lower product yield resulting from coke combustion.

Applicant has now found a process in which these disadvantages may be avoided.

The invention relates to a process for calcining green coke containing combustible volatile matter in at least two stages, whereby in a first stage the green coke is heated in a furnace to a temperature of between 750°C and 1000°C and in a second stage in a second furnace to a temperature of between 1200°C and 1600°C, characterized in that the heating in the first stage is carried out with a controlled heat-up rate of less than 60°C/min in the temperature range of between 600°C and 800°C, whereby said heating up is achieved by hot combusted volatile matter, which is obtained by withdrawing the released volatile matter from the first stage, burning said volatile matter outside the first stage and recycling the burnt volatile matter to the first stage. Part of the hot combusted gases may be obtained by burning an additional combustible gas outside the first stage and introducing the burnt gas into the first stage.

A major advantage of the process according to the invention is that the calcined coke contains sufficient coarse material, which makes it especially suitable for the manufacture of ultra high power electrodes.

It is advantageous to carry out the first stage, namely the precalination in a non-oxidising atmosphere, this means that except from some oxygen leaked into the kiln because it works below atmospheric pressure, there is no more or hardly any free oxygen present in the recycled gases. The atmosphere in the precalcination stage could also be described as reducing.

In principle in the first stage any type of furnace is suitable, a rotary kiln is preferred. In the second stage any type of kiln may be suitable. Preference is given to the combination of a rotary kiln with a rotary hearth furnace in the first and second stage respectively.

The heat-up rate control in the first stage is regulated by the temperature and the amount of combusted gases, which preferably flow countercurrently with the direction in which the green coke flows. In a rotary kiln the direction in which the green coke flows, has a small angle with the horizontal surface. The inclination of said rotary kiln is generally below 5°. Depending upon the total length and the rotational speed of the kiln the retention time of the coke in the first kiln may be so chosen that the heat-up rate does not exceed 60°C per minute, preferably the heat-up rate is less than 40°C per minute. At the upper part of the rotary kiln the green coke is introduced and due to the rotation of the kiln and the gravity the green coke moves to the lower end of the kiln. The combustible volatile matter released from the green coke in the first stage, leaves the upper end and is recycled via a burner to the first stage furnace. Additional combustible gas if necessary, and air are added, so that combustion takes place in the burner. The combusted gases entering the lower part of the kiln have a temperature of between 900°C and 1300°C. A part of the combustible volatile matter is withdrawn from the recycling system before entering the burner. The right temperature and the amount of burnt gas necessary to achieve the controlled release of the combustible gases from the green coke is in this way secured. The amount of oxygen in the air introduced into the burner, is generally completely used for combustion of the gases, before these are recycled to the furnace in the first stage. The precalcined coke leaving the lower part of the kiln is transported to a rotary hearth furnace or other kiln. The kilns of the first and the second stage may be so arranged that the transport takes place by gravity. The inlet of the calciner may be positioned immediately below the outlet of the precalciner and the precalcined coke is directly dropped into the coke feeding device of the calciner. Transportation may also take place by means of a conveyor. After the green coke has been subjected to precalcination, the obtained product may preferably be cooled to a temperature below 100°C, or even to room temperature. As already stated hereinbefore the second stage (calcination) may take place in any kind of furnace, in which the presence of free oxygen may be tolerated. Preference is given to a rotary hearth furnace, which is well known in industry.

The process as applicable to any type of green coke, produced by delayed coking from heavy oils of petroleum or coal origin, such as residue oils of catalytic cracking, thermal cracking or steam cracking, straight run oils and tars resulting from thermal cracking or coal tar pitch or any suitable blend of two or more of the above-mentioned oils before or after any additional treatment as thermal treatment, solvent extraction or hydrotreatment and the like.

Furthermore, the process according to the invention may be carried out in such a way that only one furnace is used with two different stages: the precalcination and the calcination, wherein the temperatures and gas compositions are controlled.

### Example

Green coke with a water content of 9% weight was introduced at the upper end into a rotary kiln (with a length of 12 metres and an internal diameter of 0.5 metre) and precalcined to a temperature of 826°C. The green coke was introduced at a rate of 250 kg/h, while the kiln was operated at 2 rpm (rotations per minute), the inclination being 2.5 degrees. The green coke was obtained as residue in the steam cracking process of naphtha and gas oil.

The green coke was heated-up with a flue gas which had a temperature of 950°C and which gas flowed in the direction countercurrently with the direction in which the coke was moving. The outlet temperature of the flue gas was 480°C. The flue gas which contained no. free oxygen, was produced by external stoichiometric combustion in a burner chamber of 16 kg/h natural gas with 206 kg/h air of ambient temperature and quenching the adiabatic flame temperature with a recycle of 730 kg/h of the total amount of 1081 kg/h of kiln-off gas. 357 kg/h of the kiln-off gas is withdrawn from the recycle stream. 218 kg/h of precalcined coke was obtained at the lower end of the rotary kiln.

The heat-up rate of the coke in the temperature range of from 600°C to 800°C was 24°C/min.

After cooling to 20°C precalcined coke was introduced at a rate of 100 kg/h at the upper end into a second rotary kiln with a final temperature of 1380°C. This rotary kiln was operated at 3.6 rpm and had the same length and diameter as the first kiln. The inclination was 2.5 degrees. The coke was heated up by once through countercurrent heat exchange in an oxidizing atmosphere with a flue gas which had an inlet temperature of 1480°C. The flue gas was obtained by combustion of natural gas with air and additional air was added to maintain an oxidizing atmosphere in the kiln. Starting from 100 kg/h of precalcined coke 94 kg/h of calcined coke was obtained. Real density was 2.13 g/ml.

### Comparative Example

A comparative experiment was carried out in the same rotary kilns, in which the precalcination and the final calcination took place.

250 kg/h of green coke was introduced at the upper end into a rotary kiln and precalcinated, while the kiln was operated at 2 rpm.

The green coke was heated-up with a flue gas which had a temperature of 950°C and which gas flowed in the same direction as the coke was moving in the kiln. The flue gas was obtained by burning 17 kg of natural gas with 221 kg/h air of ambient temperature and was quenched with 312 kg/h additional air of ambient temperature. Burning of the released combustible gases took place in the rotary kiln. No recycle of the flue gas took place. 214 kg/h of precalcined coke was obtained.

The heat-up rate of the coke in the temperature range of from 600° to 800°C could not be controlled, when additional air was used.

The precalcined coke was calcined in the second rotary kiln under exactly the same conditions as described in the example. Starting from 100 kg/h of precalcined coke 94 kg/h of calcined coke was obtained. Real density was 2.13 g/ml.

The calcined cokes obtained by the process according to the invention (example) and the process according to the comparative example differed considerably in physical characteristics.

Hereinafter the friability of the calcined cokes will be compared.

From Table 1 it is evident that the friability of the calcined coke produced by the process according to the invention has been decreased, the coke has thus become less friable. Starting from a green coke with a given size distribution, it is observed that the obtained coke has hardly undergone any changes in size distribution in the process according to the invention.

From Table 2 it is evident that the calcined coke obtained by the process according to the invention is better proof against deterioration than the calcined coke not produced according to the invention.

From Table 3 it is evident that the calcined coke, when graphitized, and prepared by the method accoridng to our invention, has a coefficient of thermal expansion which is less than that of calcined and graphitized coke not prepared according to the invention.

## Claims

1. A process for calcining green coke containing combustible volatile matter in at least two stages, whereby in a first stage the green coke is heated in a furnace to a temperature of between 750°C and 1000°C and in a second stage in a second furnace to a temperature of between 1200°C and 1600°C, characterized in that the heating in the first stage is carried out with a controlled heat-up rate of less than 60°C/min in the temperature range of between 600°C and 800°C, whereby said heating up is achieved by hot combusted volatile matter, which is obtained by withdrawing the released volatile matter from the first stage, burning said volatile matter outside the first stage and recycling the burnt volatile matter to the first stage.

2. A process as claimed in Claim 1, characterized in that part of the hot combusted volatile matter is obtained by burning an additional combustible gas outside the first stage and introducing the burnt gas into the first stage.

3. A process as claimed in Claims 1-2, characterized in that in the first stage furnace a non-oxidizing atmosphere is upheld.

4. A process as claimed in Claims 1-3, characterized in that in the first stage a rotary kiln is used.

5. A process as claimed in Claims 1-4, characterized in that in the second stage a rotary hearth furnace is used.

6. A process as claimed in Claims 1-4, characterized in that in the first stage the hot combusted volatile matter is recycled countercurrently with the direction in which the green coke, being precalcined, flows.

7. A process as claimed in Claims 1-4, and 6, characterized in that the hot combusted volatile matter has a temperature of between 900°C and 1300°C.

8. A process as claimed in Claims 1-4, 6 and 7, characterized in that the amount of oxygen is completely used for combustion of the combustible volatile matter derived from the coke and the additional combustible gas, before they are recycled to rotary kiln.

9. A process as claimed in Claims 4-5, characterized in that the rotary kiln is situated above the rotary hearth furnace, enabling the coke transport taking place by gravity.

10. A process as claimed in Claims 1-9, characterized in that in the first stage the heating is carried out with a controlled heat-up rate of less than 40°C/min.

11. A process as claimed in Claims 1-10, characterized in that the precalcinated coke is cooled to a temperature below 100°C, before it is subjected to the calcination in the second stage.

## Patentansprüche

1. Verfahren zum Kalzinieren von brennbares flüchtiges Material enthaltendem grünem Koks in wenigstens zwei Stufen, wobei in einer ersten Stufe der Koks in einem Ofen auf eine Temperatur zwischen 750°C und 1.000°C erhitzt wird und in einer zweiten Stufe in einem zweiten Ofen auf eine Temperatur zwischen 1.200°C und 1.600°C erhitzt wird, dadurch gekennzeichnet, daß das Erhitzen in der ersten Stufe mit einer kontrollierten Aufheizgeschwindigkeit von weniger als 60°C/min im Temperaturbereich zwischen 600°C und 800°C ausgeführt wird, wobei dieses Erhitzen durch heißes verbranntes flüchtiges Material, das durch Abziehen des freigesetzten flüchtigen Materials aus der ersten Stufe, Verbrennen dieses flüchtigen Materials außerhalb der ersten Stufe und Rückführen des verbrannten flüchtigen Materials in die erste Stufe erhalten worden ist, vorgenommen wird.

2. Verfahren nach Anspruch 1, dadurch gekennzeichnet, daß ein Teil des heißen verbrannten flüchtigen Materials durch Verbrennen eines zusätzlichen brennbaren Gases außerhalb der ersten Stufe und Einführen des verbrannten Gases in die erste Stufe erhalten wird.

3. Verfahren nach den Ansprüchen 1 und 2, dadurch gekennzeichnet, daß im Ofen der ersten Stufe eine nicht oxidierende Atmosphäre aufrecht erhalten wird.

4. Verfahren nach einem der Ansprüche 1 bis 3, dadurch gekennzeichnet, daß in der ersten Stufe ein Drehrohrofen verwendet wird.

5. Verfahren nach den Ansprüchen 1 bis 4, dadurch gekennzeichnet, daß in der zweiten Stufe ein Rotations-Herdofen verwendet wird.

6. Verfahren nach einem der Ansprüche 1 bis 4, dadurch gekennzeichnet, daß in der ersten Stufe das heiße verbrannte flüchtige Material im Gleichstrom zur Richtung, in welcher der dem Präkalzinieren unterliegende grüne Koks strömt, zurückgeführt wird.

7. Verfahren nach den Ansprüchen 1 bis 4 und 6, dadurch gekennzeichnet, daß das heiße verbrannte flüchtige Material eine Temperatur von 900°C bis 1.300°C aufweist.

8. Verfahren nach den Ansprüchen 1 bis 4, und 7, dadurch gekennzeichnet, daß die Sauerstoffmenge völlig zur Verbrennung des vom Koks stammenden brennbaren flüchtigen Materials und des zutätzlichen brennbaren Gases verbraucht wird, bevor sie zum Drehrohrofen zurückgeführt werden.

9. Verfahren nach Ansprüchen 4 und 5, dadurch gekennzeichnet, daß der Drehrohrofen oberhalb des Rotations-Herdofens angeordnet ist, sodaß der Kokstransport zufolge der Schwerkraft stattfinden kann.

10. Verfahren nach den Ansprüchen 1 bis 9, dadurch gekennzeichnet, daß in der ersten Stufe das Aufheizen mit einer kontrollierten Aufheizgeschwindigkeit von weniger als 40°C/min ausgeführt wird.

11. Verfahren nach den Ansprüchen 1 bis 10, dadurch gekennzeichnet, daß dervorkalzinierte Koks auf eine Temperatur unter 100°C abgekühlt wird, bevor er in der zweiten Stufe der Kalzinierung unterzogen wird.

## Revendications

1. Procédé de calcination du coke vert contenant une matière combustible volatile, en au moins deux stades, qui consiste, dans un premier stade, à chauffer le coke vert dans un four à une température comprise entre 750°C et 1000°C et, dans un second stade, à le chauffer dans un second four jusqu'à une température comprise entre 1200°C et 1600°C, caractérisé en ce que le chauffage, dans le premier stade, est réalisé avec une vitesse de montée en température contrôlée de moins de 60°C par minute dans l'intervalle de température compris entre 600°C et 800°C, cette montée en température étant obtenue grâce à de la matière volatile brûlée, que l'on obtient en soutirant la matière volatile libérée du premier stade, en brûlant cette matière volatile en dehors du premier stade et en recyclant la matière volatile brûlée vers le premier stade.

2. Procédé selon la revendication 1, caractérisé en ce que l'on obtient une partie de la matière volatile brûlée chaude en faisant brûler un gaz combustible additionnel en dehors du premier stade et en introduisant le gaz brûlé dans le premier stade.

3. Procédé selon les revendications 1-2, caractérisé en ce que l'on maintient, dans le four du premier stade, une atmosphère non oxydante.

4. Procédé selon les revendications 1-3, caractérisé en ce que l'on utilise, dans le premier stade, un four rotatif.

5. Procédé selon les revendications 1-4, caractérisé en ce que l'on utilise, dans le second stade, un four à sole rotative.

6. Procédé selon les revendications 1-4, caractérisé en ce que, dans le premier stade, la matière volatile brûlée chaude est recyclée à contre-courant par rapport au sens d'écoulement du coke vert pendant sa précalcination.

7. Procédé selon les revendications 1-4 et 6, caractérisé en ce que la matière volatile brûlée chaude a une température comprise entre 900°C et 1 300°C.

8. Procédé selon les revendications 1-4, 6 et 7, caractérisé en ce que la quantité d'oxygène est intégralement utilisée pour la combustion de la matière combustible volatile dérivée du coke et du gaz combustible additionnel, avant leur recyclage vers le four rotatif.

9. Procédé selon les revendications 4-5, caractérisé en ce que le four rotatif est situé au-dessus du four à sole rotative, ce qui permet au transport du coke de se faire par gravité.

10. Procédé selon les revendications 1-9, caractérisé en ce que, dans le premier stade, le chauffage est réalisé avec une vitesse de montée en température contrôlée inférieure à 40°C/min.

11. Procédé selon les revendications 1-10, caractérisé en ce que le coke précaliné est refroidi à une température inférieure à 100°C avant d'être soumis à la calcination dans le second stade.
